

J. W. NESMITH.  
BLAST FURNACE SMELTING.  
APPLICATION FILED JUNE 12, 1908.

910,082.

Patented Jan. 19, 1909.

Fig. 1.



Fig. 2.



Attest.  
Bent, Stahl.  
Edward N. Sartor

Inventor:  
John W. Nesmith,  
By Oscar Middleton, Donaldson & Son,  
Atty's.

# UNITED STATES PATENT OFFICE.

JOHN W. NESMITH, OF DENVER, COLORADO, ASSIGNOR TO COLORADO IRON WORKS COMPANY, OF DENVER, COLORADO.

## BLAST-FURNACE SMELTING.

No. 910,082.

Specification of Letters Patent.

Patented Jan. 19, 1909.

Application filed June 12, 1908. Serial No. 438,114.

*To all whom it may concern:*

Be it known that I, JOHN W. NESMITH, citizen of the United States, residing at Denver, Colorado, have invented certain new and useful Improvements in Blast-Furnace Smelting, of which the following is a specification.

My invention herein described relates to the treatment of oxidized ores.

10 The invention is an improvement in the smelting method as heretofore practiced and consists in supplying heat generated outside the furnace, to the shaft thereof, preferably from crude petroleum or gas, the heat thus supplied being utilized in lieu of the solid carbonaceous fuel, as coke, charcoal or their equivalents theretofore used. The method includes supplying air to the furnace, independently of the heat generated outside and forced into the furnace.

An apparatus for carrying the invention into effect is illustrated in the accompanying drawing, in which the figure is a sectional view.

25 I utilize a blast furnace shaft of the same general design as those in common use for pyrite smelting or copper matting, and, with some modifications, for lead smelting, and having auxiliary thereto a fire-box or combustion chamber of suitable proportions for burning the necessary quantity of crude oil or petroleum, to supply an adequate equivalent of heat to the shaft of the furnace into which the ores and fluxes for smelting are charged, to consummate the smelting continuously to completion as such ores and fluxes are charged in, the heat from the crude oil or petroleum being used instead of coke, or other solid carbon, as fuel only, in oxidizing smelting and not for producing any other reactions involved.

The oil or gas fuel in this system is burned in a fire box or combustion chamber, segregated entirely as to combustion from the ores and fluxes being smelted in the blast furnace, so that the chemical reactions incident to the combustion of carbonaceous fuel for the production of heat necessary for smelting shall not take place in contact with the ores being smelted, in order to avoid the complications involved in burning carbonaceous fuel in contact with the ores and fluxes or with the air blast in a smelting operation whose necessary reactions are wholly oxidizing, as in smelting sulfid ores to a regulus or matte product

Air is blown into such a furnace for the purpose of furnishing the oxygen necessary to oxidize the waste materials, as the sulfur and the iron of the sulfid ores, the latter to iron oxid to combine with the silica in the ore 60 to form a fluid slag to flow freely away to the dump, the sulfur up the chimney to the atmosphere.

Oxygen has a stronger affinity for carbonaceous fuel, as coke or charcoal or oil, than it 65 has for iron or sulfur, and hence when such carbonaceous fuel as coke or charcoal or oil is charged into the furnace with the ores, or as oil is burned in the air blast of the furnace, no reaction can take place of oxygen with 70 iron and sulfur until the carbonaceous fuel has been fully satisfied with oxygen or unless there is a surplus of oxygen going into the furnace over and above that demanded by the carbonaceous fuel. In other words, 75 the combustion of carbonaceous fuel in the atmosphere of the blast furnace smelting to a matte product, is essentially counteractive of the oxidizing reactions involved in such smelting methods, and hence the use of car- 80 bonaceous fuel burning in contact with ores being smelted, under the action of the air blast is entirely avoided in this method.

In my improved method the heat, necessary to be supplied to the smelting furnace, 85 is produced by burning oil or gas to its ultimate products of combustion in a combustion chamber outside of the blast furnace where the ore is smelted, and the heat so produced is conveyed by convection through 90 suitable ducts together with the inert gases of combustion, into the smelting furnace, and so the necessary heat for smelting the ores is supplied to the furnace without the counteractive effect involved where carbona- 95 ceous fuel is burned in the atmosphere of the furnace or in contact with the ores being smelted.

In some cases, so much coke or other hard carbon is used in the furnace stack with the 100 ores as is necessary to the reducing reaction from oxid to metal or other necessary reactions of such nature involved in such reducing smelting, but no hard carbon is used in the furnace stack for producing heat, or 105 for other purposes than that named above.

In the drawings, A is a blast furnace of usual construction, having twyers B. A fire box or combustion chamber is shown at C, in which petroleum or other fluid or gaseous 110

hydrocarbon is burned for the production of heat.

H is a pipe leading from a blower of usual construction furnishing air to the chamber 5 C, in quantity sufficient to maintain complete combustion of the oil or gas in the fire box and under pressure sufficient to force the heat and products of combustion from the chamber into the smelting furnace. A 10 duct or flue D connects the furnace with the combustion chamber C, through which the heat, with the products of combustion generated in the fire box are forced directly into the blast furnace against the pressure, if 15 any, maintained in the blast furnace stack A by the air blast from the blower supplying the twyters.

E is a general form of bustle pipe with an air duct F delivering the air blast from a 20 blower necessary to the process of smelting the ores in the stack. One form of such air duct F (Fig. 2) is made as a slot or rectangular opening parallel with the plane of the furnace hearth, and preferably of such 25 proportions as to admit the full blast of air from the blower G without constriction, as is involved in the use of the twyters B shown in Fig. 1 and commonly employed at the entrance to the furnace. Some air may be 30 necessary in the reducing furnace for such office, among other things, as producing carbon monoxid from coke or charcoal charged on with the ores for reducing oxids to metals.

The twyters B or the air blast duct F, as 35 the case may be, and the heat duct D in the form shown, enter the furnace A preferably in so near proximity to each other that the heat and heated gases from the combustion

chamber C meet and commingle with the air blast, if any, within the blast furnace, 40 thus warming or heating the air blast immediately on its entrance and avoiding the paralyzing effect of cold air in the smelting zone, while at the same time the heat over and above that utilized for heating the air 45 in the blast furnace A necessary for the smelting operation, is provided through the heat duct D from the combustion chamber C.

In this method of smelting to lead base 50 bullion or other metals, it is also convenient to use liquid or gaseous fuel as a reducing agent, to which the air may be accurately supplied in such proportions as to produce carbon monoxid and thus secure perfect and complete reduction of oxids to their metals. 55

I claim:—

The herein described method of treating oxidized ores, which consist in feeding a mixture of ores and fluxes and such carbonaceous material as is necessary for the reactions involved in the reduction of such ore to metals into a blast furnace, burning a suitable fuel exterior to the blast furnace and passing the hot combusted products into the blast furnace to supply the heat necessary 60 for the reduction of the ore, and supplying air to said furnace independently of said combusted products to furnish the oxygen necessary for the proper reduction of the ore.

In testimony whereof, I affix my signature 70 in presence of two witnesses.

JOHN W. NESMITH.

Witnesses:

WINTHROP R. CADY,  
H. B. LOWDEN.